

1,163,271.

G. B. SHIPLEY.

METHOD OF FIREPROOFING TIMBER.

APPLICATION FILED APR. 5, 1915.

Patented Dec. 7, 1915.



WITNESSES

*W.T. Johnson*  
W. T. Johnson  
W. B. Wharton

INVENTOR

*Grant B. Shipley*  
By *Frank M. Winter*  
Attorneys

GRANT B. SHIPLEY, OF PITTSBURGH, PENNSYLVANIA.

## METHOD OF FIREPROOFING TIMBER.

1,163,271.

Specification of Letters Patent. Patented Dec. 7, 1915.

Application filed April 5, 1915. Serial No. 19,286.

*To all whom it may concern:*

Be it known that I, GRANT B. SHIPLEY, a resident of Pittsburgh, in the county of Allegheny and State of Pennsylvania, have invented a new and useful Improvement in Methods of Fireproofing Timber, of which the following is a specification.

This invention relates to a method of fireproofing timber, and more particularly relates to the treatment of shingles and building timber, with an antiseptic for the preservation of the timber and with a fireproofing substance, the treatment with the two substances preferably being simultaneous.

10 The main object of the invention is to provide a method for treating shingles and other timbers, whereby cementitious and silicious material is forced into the pores of the wood to be treated, thereby effectually fireproofing the same.

15 A further object of the invention is to provide a method wherein this fireproofing treatment is carried out simultaneously with the treatment of the wood with a preservative so that by a single process the wood can be protected against rotting as well as against danger from fire.

20 The cementitious material forced into the wood not only acts as an efficient fireproofing, but when a preserving solution is forced into the wood either previously to or simultaneously with the application of the cementitious material, it will prevent leaching out or evaporation of the preserving solution, 25 and will in itself greatly strengthen the timber which has been treated. The fireproofing treatment will also to a great extent prevent expansion and contraction of timbers to which it has been applied.

30 It is of great importance both owing to fire regulations and from general considerations of safety that wood used as building material be effectually fireproofed, and that the fireproofing process used be sufficiently cheap to allow its application under all ordinary conditions. Methods of fireproofing wood as heretofore employed have been either only slightly effectual or of a nature which involves expense, and are often not 35 applicable to wood as used in general building. One method heretofore used has been the application of a mixture of cement and sand to the wood to be fireproofed by means of a cement gun. This method does not cause the material to penetrate to any great 40 extent into the pores of the wood, and if a

coating sufficient to thoroughly fireproof the wood is applied by this means the resulting timbers are made heavy and hard to handle.

45 By means of the present method a quantity of cementitious material either alone or together with a preservative solution is forced into the cellular structure of timber being treated and forms an impermeable protective layer which lies chiefly within the body of the wood and thoroughly fireproofs 55 the same. This coating material is applied under pressure to secure the desired result, and the wood is preferably treated at the same time with a preserving solution. In 60 this case the preserving material being in solution will be forced a considerable distance into the wood, while the cementitious material will be forced a lesser distance into 65 its cellular structure.

70 The preferred materials used in this method consist of zinc chlorid as a preservative and a mixture of cement together with fine or pulverized sand or some suitable infusorial earth, such as kieselguhr all 75 ground to an impalpable powder. It has been found that the proportion of material giving the best results are about one half pound of dry zinc chlorid for each cubic foot of timber to be treated, and cement and sand or infusorial earth to the amount desired, the proportion of the latter being one part of cement to from four to six parts of sand or infusorial earth.

80 The method may be carried out by various forms of apparatus, and the accompanying drawing shows merely diagrammatically a single form or arrangement of apparatus by means of which the method may be carried out. The apparatus may be 85 of any design, but as illustrated comprises a suitable treating cylinder shown at 1, in which the timber is treated; a storage tank 2 in which the zinc chlorid solution is mixed with the cementitious material; a pressure 90 pump 3; suitable connections between the same comprising pipe 4 leading from the storage tank to the treating cylinder; a pipe 5 between the pressure pump and storage tank; and suitable means for agitating the 95 mixture in the treating cylinder.

100 In carrying out the method, wood which has been properly seasoned is placed in the treating cylinder which is then sealed. The treating bath is formed by introducing into 105 the storage tank either a solution of zinc chlorid and adding cement and pulverized

sand or infusorial earth thereto, or by dissolving the zinc chlorid and mixing with the solid material at a single step. The bath may be stirred to cause the solid materials to be suspended therein and is then passed by gravity or by the pressure of pump 3 into the treating cylinder. When the treating cylinder 1 has been charged with the wood and the treating and fireproofing bath, pressure up to about 200 pounds is applied by means of pump 3. Both the preserving solution and the cementitious material together with its body of sand or infusorial earth will be forced into the cells of the wood. The zinc chlorid, however, being in solution will pass first into the wood and will penetrate farther therein than the solid material, in the case of shingles and light boards completely saturating the wood. The cement and other solid material is forced only a short distance into the wood, but completely fills the pores thereof to the limit of its penetration, leaving merely a light coating upon the surface of the wood. Since the cement and sand or infusorial earth do not remain evenly distributed throughout the body of the liquid, under ordinary conditions, it is necessary to provide means to cause a continuous agitation of the bath in order that these particles may be held in even suspension through the bath during the process of forcing them into the cellular structure of the wood being treated. This may be accomplished by any suitable means but as shown in the drawing is by means of a circulating system. In this system a pipe 6 leads from a plurality of openings 7 in the top of the treating cylinder to a centrifugal pump 8 connected by conduit 9 with a perforated pipe 10 in the bottom of the treating cylinder and extending entirely therewith. By this means fluid is continuously withdrawn during the treating process from the top of the treating cylinder and is forced by the pump into the cylinder through the perforated pipe 10 so that the liquid is continuously agitated throughout the length of the cylinder, thereby keeping the particles properly mixed and in suspension during treatment of the wood.

Preferably, the storage tank 2 is elevated above the treating cylinder 1 so that the treating mixture will flow by gravity into the treating cylinder. Suitable scales 11 upon which the storage tank 2 rests are also provided so that the quantity of mixture absorbed during treatment can be easily determined. While in the drawing only a single treating cylinder is shown as supplied from the storage tank, it is obvious that any desired number of such cylinders can be connected to a single storage tank by a suitable system of piping.

Since the fireproofing as applied by this method penetrates the pores of the wood, it

cannot be impaired by chipping or by the entrance of water into the protective coating. It prevents splitting and checking of the timber, and also prevents warping, which is of particular importance when it is applied to shingles.

The most important use of the fireproofing method described is in the fireproofing of shingles since they are most greatly subjected to fire dangers. It is also, however, applicable to building timbers in general, and may be advantageously used for the treatment of paving blocks and cross ties where its hardening and strengthening qualities, and its effect in preventing expansion and contraction of the wood, are of particular advantage. Piles upon treatment with cement by this method are protected against splitting during the operation of driving, and are protected from attack by insects or marine borers.

The method described is economical, since only so much fireproofing material is required as will effectually close the pores of the timber treated, and a heavy deposit of the material is not permitted to form upon the surface of the wood. The wood is also much lighter than if a heavy layer of cement were applied thereto externally.

It is to be understood that the method is not limited to the simultaneous treatment of timbers with preservatives and fireproofing substances, but that methods comprising merely a fireproofing treatment, or successive treatments first with a preservative and then with a fireproofing material, are within the scope of the claims hereto appended.

What I claim is:—

1. The process of treating wood consisting in forcing cementitious material into the pores thereof.

2. The process of treating wood consisting in forcing into the pores thereof a preserving solution and cementitious material.

3. The process of treating wood consisting in simultaneously forcing a preserving solution and cementitious material into the pores thereof.

4. The process of treating wood consisting in subjecting the same to a bath containing cementitious material in suspension under a pressure higher than atmospheric pressure, and agitating the bath during treatment of the wood.

5. The process of treating wood consisting in subjecting the same to a bath containing cementitious material and pulverized silicious material in suspension under a pressure higher than atmospheric pressure, and agitating the bath during the treatment to maintain the cementitious and silicious materials in suspension.

6. The process of treating wood consisting in subjecting the same to a bath containing cementitious material and pulverized infu-

sorial earth in suspension under a pressure higher than atmospheric pressure, and agitating the bath during the treatment to maintain the cementitious material and infusorial earth in suspension.

7. The process of treating wood consisting in subjecting the same to a bath containing a preservative in solution and cementitious material in suspension under a pressure higher than atmospheric pressure, and agitating the bath during treatment of the wood.

8. The process of treating wood, consist-

ing in subjecting the same to a bath containing zinc chlorid in solution and cementitious material in suspension under a pressure higher than atmospheric pressure, and agitating the bath during treatment of the wood.

In testimony whereof, I have hereunto set my hand.

GRANT B. SHIPLEY.

Witnesses:

WILLIAM B. WHARTON,  
GLENN H. LERESCHE.